

# UNITED STATES PATENT OFFICE.

GUSTAF W. ELMEN, OF LEONIA, NEW JERSEY, ASSIGNOR TO WESTERN ELECTRIC COMPANY, INCORPORATED, OF NEW YORK, N. Y., A CORPORATION OF NEW YORK.

## MAGNET CORE AND METHOD OF MAKING THE SAME.

1,403,305.

Specification of Letters Patent. Patented Jan. 10, 1922.

No Drawing.

Application filed December 21, 1920. Serial No. 432,357.

To all whom it may concern:

Be it known that I, GUSTAF W. ELMEN, a citizen of the United States, residing at Leonia, in the county of Bergen and State of New Jersey, have invented certain new and useful Improvements in Magnet Cores and Methods of Making the Same, of which the following is a full, clear, concise, and exact description.

10 This invention relates to magnet cores and particularly to telephone loading-coil cores of the so-called "dust" type, such as are described in the patent issued in my name, No. 1,297,126, dated March 11, 1919, 15 and the other patents therein referred to.

The general object of the present invention is to obtain a new and improved magnet core which is cheap to manufacture and possesses to a high degree, those characteristics that are desirable in cores for loading coils and other electrical apparatus.

The present invention is broadly characterized by the treatment of finely divided magnetic material with a carbonizing agent 25 for the purpose of hardening it. Hardened finely divided magnetic material so obtained is particularly suitable for the manufacture of cores for loading coils and other telephone apparatus, by reason of the low 30 hysteretic losses which will exist in such cores when subjected to the influences of telephonic currents.

The present method is applicable to any 35 of the magnetic metals, iron, nickel and cobalt. It will, however, be described as applied to iron since this is the magnetic material most usually employed for magnet cores.

The iron to be used may be either in the 40 form of finely divided iron such, for example, as what is commercially known as "iron-by-hydrogen;" or, in the form of iron oxide. In either case, the material is treated with a carbonizing agent such as carbon or an hydrocarbon, sufficient heat being applied to 45 facilitate the reducing and carbonizing process. Preferably, iron oxide is used, and with this is mixed enough finely divided carbon not only to reduce the oxide but also to combine with the reduced metal. This mixture of finely divided iron oxide and carbon 50

is heated to a temperature below the melting temperature of the metal but high enough to cause the reduction of the iron by the carbon and the combining of the excess carbon with

the reduced metal. Such a temperature is 55 about 300° to 400° C. below the melting temperature of iron. This reducing and carbonizing treatment causes the material to take a spongy form from which it may be reduced to a finely divided state by grinding. 60

The hard iron particles so obtained may be sorted by sifting, coated with insulating material, and formed into a solid in the usual manner as described in the patents hereinbefore mentioned. 65

What is claimed is:

1. The method of making magnet cores which consists in treating finely divided magnetic material with a carbonizing agent, 70 coating the particles with insulating material, and forming a mass of such particles into a solid.

2. The method of making magnet cores which consists in treating iron in finely divided form with a carbonizing agent, coating the particles with insulating material, 75 and forming a mass of such particles into a solid.

3. The method of making magnet cores which consists in heating to a carbonizing 80 temperature a mixture of finely divided magnetic material and carbon, coating the particles with insulating material, and forming a mass of such particles into a solid.

4. The method of making magnet cores 85 which consists in heating to a carbonizing temperature finely divided iron and finely divided carbon, coating the particles with insulating material, and forming a mass of such particles into a solid. 90

5. The method of making magnet cores which consists in treating an oxide of a magnetic metal with a reducing and carbonizing agent, grinding up the resulting product, 95 coating the particles thus obtained with insulating material, and forming a mass of such particles into a solid.

6. The method of making magnet cores which consists in treating an iron oxide with a reducing and carbonizing agent, grinding 100 up the resulting product, coating the particles thus obtained with insulating material, and forming a mass of such particles into a solid.

7. The method of making magnet cores 105 which consists in heating to a reducing and carbonizing temperature a mixture of iron oxide and carbon, grinding up the resulting

product, coating the particles thus obtained with insulating material, and forming a mass of such particles into a solid.

8. A magnet core composed of finely divided magnetic material hardened by treatment with a carbonizing agent, and insulating material separating the particles of magnetic material.
9. A magnet core composed of finely di-

vided iron hardened by heating to a carbonizing temperature with finely divided carbon, and insulating material separating the particles of magnetic material.

In witness whereof, I hereunto subscribe my name this 20th day of December A. D., 1920.

GUSTAF W. ELMEN.